

Feb. 18, 1936.

M. HAGEDORN ET AL

2,030,983

TREATMENT OF FILMS AND FOILS OF ORGANIC CELLULOSE ESTERS

Filed Oct. 3, 1932

Fig. 1



Fig. 2



Inventors:  
M. Hagedorn,  
Paul Mueller,  
Philip S. Hopkins.  
By Attorney

## UNITED STATES PATENT OFFICE

2,030,983

TREATMENT OF FILMS AND FOILS OF  
ORGANIC CELLULOSE ESTERS

Max Hagedorn, Dessau in Anhalt, and Paul Möller, Dessau-Ziebigk, Germany, assignors to Agfa Ansco Corporation, Binghamton, N. Y., a corporation of New York

Application October 3, 1932, Serial No. 636,074  
In Germany October 5, 1931

14 Claims. (Cl. 18—57)

Our present invention relates to a process of treating films and foils of organic cellulose esters and more particularly to the superficial saponification of such films and foils.

5 One of its objects is an improved process of saponifying films or foils of organic cellulose ester containing a softening agent. Further objects will be seen from the detailed specification following hereafter.

10 In the accompanying drawing there are shown foils embodying our invention. Fig. 1 shows a conventional exaggerated cross-sectional view of a foil made of a cellulose derivative and saponified on both faces. Fig. 2 shows a like view of a foil provided on one face with a photographic emulsion layer and saponified on the other.

A preliminary treatment of a cellulose acetate film to which a photographic gelatine emulsion is to be applied, consists in superficially saponifying one of its faces, so that this face shall be more or less completely regenerated to cellulose in order to ensure a good adhesion between the film and the layer of applied emulsion. This treatment produces a certain improvement of the mechanical properties of the film, but not one of practical importance, the elongation in water of the saponified material being at the same time considerably increased. Elongation in water means the percentage increase in length of a strip of the film immersed for one hour in water at 18° C.

30 According to this invention films and foils of considerably improved mechanical properties and a sensitiveness to water which is not greater than that of existing commercial films of cellulose derivatives, are obtained by conducting the saponifying treatment in a particular way which will more clearly result from the following examples. The treatment renders the films suitable for use as photographic supports.

Furthermore we have found that it is not necessary to carry out the saponification before applying a photographic emulsion to the film. 40 The treatment is also applicable to photographic films which are still sensitive to light, but we prefer to apply in this case the treatment to those photographic films bearing a finished picture. It is surprising that the improvement of the mechanical properties of the film is not impaired by the presence of the photographic layer. The finished, that is to say the developed and fixed emulsion layer containing metallic silver is not injured by the treatment. In order to 50 secure that the distances of the perforation holes

and their size remain unchanged, the saponification, washing and drying may be performed under tension.

The invention is applicable to films of a cellulose ester, mixed ester or ether-ester of an aliphatic carboxylic acid having up to 5 carbon atoms, the film containing a known softening agent, advantageously in an amount of more than 15 per cent and preferably in an amount of 25 to 35 per cent, calculated on the cellulose derivative. The saponification is performed with a solution of an alkali metal hydroxide or ammonium hydroxide which solution acts as a swelling agent for the film forming colloid, and is carried out rapidly in about 2½ to 15 minutes, 10 at ordinary temperature. The solvent for the saponifying agent must be miscible with water and must not react with the hydroxide to be dissolved therein. Suitable solvents are, for instance, methanol, ethyl alcohol, dioxane and glycolmonomethyl ether which are all used in their aqueous solution. On account of its property of swelling the film forming colloid, the alkaline liquid penetrates rapidly into the film. The most suitable concentration of the saponifying solution with regard to the proportion of its constituents can easily be determined by a few experiments. When the saponifying treatment, 15 which may be applied to one or both faces of the film, has penetrated to at least one sixth of the thickness of the film, it is interrupted and by a washing liquid having no solvent action on the softening agent, the last residues of the alkaline liquid are removed from the film. In the washing operation also those parts which have been 20 liberated in the saponifying treatment are removed. 25

As a washing liquid there is preferably used a mixture of two liquids, one of these liquids being a solvent for the hydroxide used and the products of saponification, and the other liquid preventing the dissolution of the softening agent. A mixture of alcohol and water has, for instance, proved useful. In this case alcohol is the solvent 30 for the hydroxide and the saponification products and water, when added in a suitable amount prevents the dissolution of the softening agent.

As softening agents all those that are known for organic cellulose derivatives are suitable, but 40 also resin, artificial resin or the like, provided that they are at least partially soluble in the saponifying liquid or are rendered soluble by action of this liquid.

The film treated according to the invention has 50

good mechanical properties. It consists either of a layer of saponified cellulose derivative and a layer of non-saponified cellulose derivative, or of two outer layers of saponified cellulose derivative and an inner layer of non-saponified cellulose derivative. The layers are interjoined at

Example 3.—A film of cellulose triacetate containing about 30 per cent of toluene sulfamide as softening agent, is saponified on both sides at 25° C. with a solution of 10 per cent strength of caustic soda in aqueous methanol (water : methanol = 1:1).

| 10                             | Softening agent | Thickness | Tenacity | Elongation | Elongation in water | Saponified layer on both sides |             | 10 |
|--------------------------------|-----------------|-----------|----------|------------|---------------------|--------------------------------|-------------|----|
|                                |                 |           |          |            |                     | Thickness                      | Acetic acid |    |
|                                | Percent         | $\mu$     | Kilos    | Percent    | Percent             | $\mu$                          | Percent     |    |
| Before treatment.....          | 40              | 175       | 100      | 20.0       | 0.5                 | 25                             | 62.3        |    |
| Saponified for 2½ minutes..... |                 | 100-120   | 130      | 23.2       | 0.72                |                                | 10          |    |
| Before treatment.....          | 30              | 170       | 105      | 18.0       | 0.6                 |                                | 62.3        | 15 |
| Saponified for 2½ minutes..... |                 | 120-130   | 144      | 18.7       | 0.59                | 13                             | 8           |    |
| 4 minutes.....                 |                 | 135-140   | 120      | 27.5       | 0.87                | 17                             | 10          |    |
| 5 minutes.....                 |                 | 120       | 128      | 24.0       | 0.82                | 19                             | 11          |    |

their contact surfaces without formation of sharp boundaries so that the film does not tend to split up. The saponified layer, amounting to at least one sixth of the thickness of the film, reveals the very strong action of the saponifying liquid, which considerably surpasses the superficial saponification obtainable by the known method.

To the expert in the cellulose industry it is surprising that in the process of this invention the elongation in water which, as a rule, increases commensurately with increased saponification of the film, becomes to a certain degree independent of the saponification. The elongation in water of films treated by this invention is generally less than 1.5 per cent.

The following examples illustrate the invention:

Example 1.—A film of cellulose triacetate containing about 25 per cent of vinyl-octadecyl ether as softening agent, is treated at 25° C. with a solution of 10 per cent strength of caustic soda in aqueous methanol (water : methanol = 1 : 1).

| 45                          | Softening agent | Thickness | Tenacity | Elongation | Elongation in water | Thickness of the saponified layer |       | 35 |
|-----------------------------|-----------------|-----------|----------|------------|---------------------|-----------------------------------|-------|----|
|                             |                 |           |          |            |                     | $\mu$                             | Kilos |    |
| Before treatment.....       | Percent         | $\mu$     | Kilos    | Percent    | Percent             |                                   |       |    |
| Treated for 10 minutes..... | 17              | 100       | 97       | 10.8       | 0.65                |                                   |       |    |
|                             | 11.5            | 85        | 114      | 16.6       | 0.99                |                                   |       |    |

After the saponification the film is washed for about 3 minutes with diluted acetic acid of 3 per cent strength and then for 15 minutes with an aqueous solution of methanol of 50 per cent strength. After treatment the film has a content of softening agent of about 10.4 per cent.

Example 2.—A film of cellulose triacetate containing about 25 per cent of urea-formaldehyde resin as softening agent, is treated at 25° C. with a solution of 10 per cent strength of caustic soda in aqueous methanol (water : methanol = 1 : 1).

| 65                         | Softening agent | Thickness | Tenacity | Elongation | Elongation in water | Thickness of the saponified layer |       | 60 |
|----------------------------|-----------------|-----------|----------|------------|---------------------|-----------------------------------|-------|----|
|                            |                 |           |          |            |                     | $\mu$                             | Kilos |    |
| Before treatment.....      | Percent         | $\mu$     | Kilos    | Percent    | Percent             |                                   |       |    |
| Treated for 4 minutes..... | 20              | 125       | 105      | 12.0       | 0.38                |                                   |       |    |
|                            | 12              | 110-120   | 138      | 16.7       | 0.37                |                                   |       |    |

After the saponification the film is washed for about 3 minutes with diluted acetic acid of 3 per cent strength and then for 15 minutes with an aqueous solution of methanol of 50 per cent strength. After treatment the film has a content of softening agent of about 12 per cent.

After the saponification the film is washed for about 3 minutes with diluted acetic acid of 3 per cent strength and then for 15 minutes with an aqueous solution of methanol of 50 per cent strength. After treatment the film has a content of softening agent of about 14.3 per cent.

Example 4.—A film of hydrolyzed cellulose acetate (56.7 per cent of acetic acid) containing 24 per cent of toluene sulfonamide and 6 per cent of diethyl phthalate is saponified at 24° C. for 5 minutes in a caustic potash solution of 9 per cent strength (water : methanol = 1:4).

|                       | Thickness | Tenacity | Elongation | Elongation in water | Thickness of the saponified layer | Thickness of the saponified layer |       | 35 |
|-----------------------|-----------|----------|------------|---------------------|-----------------------------------|-----------------------------------|-------|----|
|                       |           |          |            |                     |                                   | $\mu$                             | Kilos |    |
| Before treatment..... | Percent   | $\mu$    | Kilos      | Percent             | Percent                           |                                   |       |    |
| After treatment.....  | 78        | 150      | 78         | 28.3                | 0.75                              |                                   |       |    |
|                       | 120       | 112      | 112        | 32.5                | 1.00                              |                                   |       |    |
|                       |           |          |            |                     |                                   |                                   |       | 50 |

After the saponification the film is washed for about 3 minutes with diluted acetic acid of about 3 per cent strength and then for 15 minutes with an aqueous solution of methanol containing 60 per cent of methanol. After treatment the film has a content of softening agent of about 5 to 7 per cent.

Example 5.—A foil of cellulose acetate-butylate, containing as softening agent 25 per cent carbamic acid ethyl ester, is saponified at 24° C. for 10 minutes in a methanolic caustic soda solution of 10 per cent strength:

|                       | Thickness | Tenacity | Elongation | Elongation in water | Thickness of the saponified layer | Thickness of the saponified layer |       | 60 |
|-----------------------|-----------|----------|------------|---------------------|-----------------------------------|-----------------------------------|-------|----|
|                       |           |          |            |                     |                                   | $\mu$                             | Kilos |    |
| Before treatment..... | Percent   | $\mu$    | Kilos      | Percent             | Percent                           |                                   |       |    |
| After treatment.....  | 75        | 150      | 75         | 27.5                | 0.5                               |                                   |       |    |
|                       | 105       | 130      | 105        | 35.0                | 0.95                              |                                   |       |    |
|                       |           |          |            |                     |                                   |                                   |       | 40 |
|                       |           |          |            |                     |                                   |                                   |       | 65 |

After the saponification the film is washed for about 3 minutes with diluted acetic acid of 3 per cent strength and then for 15 minutes with an aqueous solution of methanol of 50 per cent strength.

Example 6.—A film of oxyethylcellulose acetate containing 30 per cent of ethyl acetanilide is saponified at 23° C. for 8 minutes in a caustic

soda solution (water : methanol=1:1) of 10 per cent strength.

| 5  | Thickness                             | Tenacity                            | Elongation              | Elongation in water     | Thickness of the saponified layer |
|----|---------------------------------------|-------------------------------------|-------------------------|-------------------------|-----------------------------------|
| 10 | $\mu$<br>150<br>Before treatment..... | Kilos<br>73<br>After treatment..... | Percent<br>25.0<br>28.0 | Percent<br>0.60<br>0.85 | $\mu$<br>35                       |
| 10 | 120                                   | 100                                 |                         |                         |                                   |

After the saponification the film is washed for about 3 minutes with diluted acetic acid of about 3 per cent strength and then for 15 minutes with an aqueous solution of methanol containing 60 per cent of methanol.

*Example 7.*—A foil of cellulose triacetate containing 40 per cent of p-tolene sulfonamide is saponified for 15 minutes at 24° C. on one face with a caustic soda solution of 10 per cent strength in equal parts of water and methanol.

| 25 | Thickness                             | Tenacity                            | Elongation            | Elongation in water   | Thickness of the saponified layer |
|----|---------------------------------------|-------------------------------------|-----------------------|-----------------------|-----------------------------------|
| 30 | $\mu$<br>170<br>Before treatment..... | Kilos<br>95<br>After treatment..... | Percent<br>22<br>25.1 | Percent<br>0.5<br>1.0 | $\mu$<br>25                       |
| 30 | 140                                   | 109                                 |                       |                       |                                   |

After the saponification the film is washed for about 3 minutes with diluted acetic acid of 3 per cent strength and then for 15 minutes with an aqueous solution of methanol of 50 per cent strength. After treatment the film has a content of softening agent of about 15.5 per cent.

Our invention is not limited to the foregoing examples nor to the specific details given therein. The best modification of operating the treatment will be found in each case by a few experiments. Though a solution of caustic soda in aqueous methanol, as disclosed in the examples, has proved to be well suitable other hydroxides and other solvents adapted to dissolve the hydroxide and the softening agent contained in the film are suitable. We contemplate as included within our invention all such modifications as fall within the scope of the appended claims. The term sheet as used in the claims is intended to include foils of cellulose derivatives and photographic films, such as have not yet been exposed and such as have been finished by developing and fixing.

What we claim is:

1. A process which comprises treating a sheet made of a cellulose derivative selected from the group consisting of cellulose esters, mixed esters and ether-esters of an aliphatic carboxylic acid having up to 5 carbon atoms and containing a softening agent with a solution of a hydroxide selected from the group consisting of alkali metal hydroxides and ammonium hydroxide in a liquid which has a swelling action on the film forming colloid, and removing from the sheet the treating liquid by means of liquid which has no solvent action on the softening agent.

2. A process which comprises treating a sheet made of a cellulose derivative selected from the group consisting of cellulose esters, mixed esters and ether-esters of an aliphatic carboxylic acid having up to 5 carbon atoms and containing at least 15 per cent of softening agent with a solution of a hydroxide selected from the group con-

sisting of alkali metal hydroxides and ammonium hydroxide in a liquid which has a swelling action on the film forming colloid, and removing from the sheet the treating liquid by means of liquid which has no solvent action on the softening agent.

3. A process which comprises treating a sheet made of a cellulose derivative selected from the group consisting of cellulose acetate, cellulose acetate-butyrate and oxyethylcellulose acetate and containing at least 15 per cent of softening agent with a solution of a hydroxide selected from the group consisting of alkali metal hydroxides and ammonium hydroxide in a liquid which has a swelling action on the film forming colloid, and removing from the sheet the treating liquid by means of liquid which has no solvent action on the softening agent.

4. A process which comprises treating a sheet made of a cellulose derivative selected from the group consisting of cellulose acetate, cellulose acetate-butyrate and oxyethylcellulose acetate and containing about 25 to 35 per cent of softening agent with a solution of a hydroxide selected from the group consisting of alkali metal hydroxides and ammonium hydroxide in a liquid which has a swelling action on the film forming colloid, and removing from the sheet the treating liquid by means of liquid which has no solvent action on the softening agent.

5. A process which comprises treating a sheet made of a cellulose derivative selected from the group consisting of cellulose acetate, cellulose acetate-butyrate and oxyethylcellulose acetate and containing about 25 to 35 per cent of a softening agent at least partly soluble in aqueous methanol with a solution of caustic soda in aqueous methanol, and removing from the sheet the treating liquid by means of liquid which has no solvent action on the softening agent.

6. A process which comprises treating a sheet made of a cellulose derivative selected from the group consisting of cellulose acetate, cellulose acetate-butyrate and oxyethylcellulose acetate and containing about 25 to 35 per cent of a softening agent at least partly soluble in aqueous methanol with a solution of caustic soda in aqueous methanol of about 50 per cent strength, and removing from the sheet the treating liquid by means of liquid which has no solvent action on the softening agent.

7. A process which comprises treating a sheet made of a cellulose derivative selected from the group consisting of cellulose acetate, cellulose acetate-butyrate and oxyethyl-cellulose acetate and containing about 25 to 35 per cent of a softening agent at least partly soluble in aqueous methanol but insoluble in aqueous ethanol with a solution of caustic soda in aqueous methanol of about 50 per cent strength, and removing from the sheet the treating liquid by means of an aqueous solution of ethanol.

8. A process which comprises treating a sheet made of cellulose triacetate and containing about 25 to 35 per cent of a softening agent at least partly soluble in aqueous methanol but insoluble in aqueous ethanol with a solution of caustic soda in aqueous methanol of about 50 per cent strength, and removing from the sheet the treating liquid by means of an aqueous solution of ethanol.

9. A process which comprises treating a sheet made of cellulose acetate containing about 52 to 57 per cent of acetic acid and containing about 25 to 35 per cent of a softening agent at least partly soluble in aqueous methanol but insoluble

in aqueous ethanol with a solution of caustic soda in aqueous methanol of about 50 per cent strength, and removing from the sheet the treating liquid by means of an aqueous solution of ethanol.

5 10. A sheet made of a cellulose derivative selected from the group consisting of cellulose esters, mixed esters and ether-esters of an aliphatic carboxylic acid having up to 5 carbon atoms and containing a softening agent, said sheet being on at least one of its faces saponified to the extent of at least one-sixth of its thickness by treatment with a saponifying solution having a swelling action on the film forming colloid and having an elongation in water of less than 1.5 per cent.

10 15. 11. A sheet made of a cellulose derivative selected from the group consisting of cellulose acetate, cellulose acetate-butyrate and oxyethyl-cellulose acetate and containing a softening agent, said sheet being on at least one of its faces saponified to the extent of at least one-sixth of its thickness by treatment with a saponifying solution having a swelling action on the film forming colloid and having an elongation in water of less than 1.5 per cent.

20 25. 12. A sheet made of cellulose triacetate containing a softening agent, said sheet being on at least one of its faces saponified to the extent of at least one-sixth of its thickness by treatment

with a saponifying solution having a swelling action on the film forming colloid and having an elongation in water of less than 1.5 per cent.

13. A sheet made of cellulose acetate containing about 52 to 57 per cent of acetic acid and containing a softening agent, said sheet being on at least one of its faces saponified to the extent of at least one-sixth of its thickness by treatment with a saponifying solution having a swelling action on the film forming colloid and having an 10 elongation in water of less than 1.5 per cent.

14. A process which comprises treating a sheet made of a cellulose derivative selected from the group consisting of cellulose esters, mixed esters and ether-esters of an aliphatic carboxylic acid 15 having up to 5 carbon atoms and containing a softening agent with a solution of a hydroxide selected from the group consisting of alkali metal hydroxides and ammonium hydroxide in a liquid which has a swelling action on the film forming 20 colloid and which is selected from the group consisting of an aqueous solution of methanol, ethyl alcohol, dioxane and glycol monoethyl ether and removing from the sheet the treating liquid by means of liquid which has no solvent action on 25 the softening agent.

MAX HAGEDORN.  
PAUL MÖLLER.